

# United States Patent [19]

Koishi et al.

[11] Patent Number: 4,902,596

[45] Date of Patent: Feb. 20, 1990

[54] TONER FOR ELECTROPHOTOGRAPHY  
WITH THE CHANGE CONTROLLING  
AGENT DISPERSED THEREIN

[75] Inventors: **Masumi Koishi, Sagamihara;**  
**Masuyuki Takada, Tokyo; Akio**  
**Kazama, Tokyo; Yukio Kawashima,**  
**Tokyo, all of Japan**

[73] Assignee: **Toyo Ink Mfg, Co., Ltd, Tokyo,**  
**Japan**

[21] Appl. No.: 138,307

[22] Filed: **Dec. 28, 1987**

[30] Foreign Application Priority Data

Jan. 16, 1987 [JP] Japan ..... 62-7618

[51] Int. Cl. 4 ..... G03G 9/10

[52] U.S. Cl. ..... 430/106.6; 430/108

[58] Field of Search ..... 430/110, 108, 106, 106.6

[56] References Cited

U.S. PATENT DOCUMENTS

3,725,118 4/1973 Fuller et al. .... 430/108  
4,395,485 7/1983 Kashiwagi et al. .... 430/110  
4,414,322 11/1983 Miyakawa et al. .... 430/108  
4,621,039 11/1986 Ciccarelli et al. .... 430/110

Primary Examiner—John L. Goodrow

Attorney, Agent, or Firm—Bucknam and Archer

[57] ABSTRACT

A toner for use in electrophotography comprising thermoplastic resin core particles (A) or colorant-embedded thermoplastic resin core particles (A') each having an average particle size of 1 to 15  $\mu\text{m}$ , a charge-controlling agent (B) and carrier particles (C) having an average particle size of 0.05 to 2.0  $\mu\text{m}$ , the charge-controlling agent (B) being carried on the carrier particles (C), and the carrier particles (C) with the agent (B) carried thereon being embedded in the surfaces of the resin core particles (A) or the colorant-embedded resin core particles (A').

9 Claims, No Drawings

TONER FOR ELECTROPHOTOGRAPHY WITH  
THE CHARGE CONTROLLING AGENT  
DISPERSED THEREIN

BACKGROUND OF THE INVENTION

1. Field of the Invention

This invention relates to toners used for the dry development of an electrostatic latent image in electrophotography.

2. Description of the Prior Art

There have heretofore been known several dry developing methods including a method using a two-component developer composed of toner particles mixed with carrier particles such as glass beads or magnetic powder, and a method using a one-component toner composed of toner particles imparted with magnetism. In addition, there has recently been proposed a method using a one-component nonmagnetic toner which is excellent in environment resistance, e.g. temperature, humidity and the like.

These conventional toners have been, in most cases, prepared by methods which comprise mixing, heating and melting thermoplastic resins, colorants such as pigments or dyes and additives such as wax, plasticizers, charge-controlling agents and the like, kneading the pigments or charge-controlling agents, changing the form of secondary agglomeration under the application of intense shearing force to primary particles, uniformly dispersing, if necessary, magnetic powder in the mixture to obtain a uniform composition, cooling and comminuting the composition and then classifying the resulting particles to obtain the toner particles.

However, the conventional methods have problems that they require a large amount of energy in the step of milling the pigment and charge controlling agent, provide the toner particles in a low yield as low as about 85% because finer toner particles are cut or removed in the step of classification, and exhibit an inevitably low productivity of toner particles although part of the removed toner particles are reused in the next production. Further, in cases where particulate toners which are different from each other in kind, particularly hue, are each produced by any conventional method using an apparatus including devices such as a kneader, grinder and dispenser, such devices must beforehand be thoroughly cleaned every time each of the toners is produced. Since the devices used in the conventional methods are considerably large in scale, the cleaning is a heavy burden to the workers.

Moreover, the toner particles so obtained are qualitatively disadvantageous in that they have the charge-controlling agent insufficiently dispersed therein and are non-uniform in size and shape and generally amorphous whereby they are individually different in frictional charging characteristics thus causing them to be stained and scattered within the copying devices. In addition, the toner particles have so low flowability that it becomes difficult to supply them smoothly with many troubles being undesirably involved.

To avoid this, there have been proposed attempts to obtain spherical toners by a spray drying or suspension polymerization process. However, the former process requires proper selection of resins which are soluble in the solution used and raises a problem as to an offset phenomenon on a fixing drum. The latter process raises

problems as to blocking and offset phenomena and is therefore not industrially used.

Further, other methods proposed include a method in which binder resin particles and coloring material particles are treated in a hot air stream (Japanese patent application Laid-Open No. 37553/1984) and a method in which a binder resin and a coloring material are deposited on the surface of a spherical resin (Japanese patent application Laid-Open No. 210368/1986). However, these methods involving heat treatment tend to cause the formation of coarse particles due to the fusion of fine particles and have not yet been put to practical use.

Conventional toners have the common disadvantage that the colorant and charge controlling agent, which exhibit their characteristic properties on the toner surface and are relatively expensive as starting materials for the toners, are not economically contained not only in the surface portion of the toner but also in the interior.

In order to solve this problem, one of the present inventors proposed a toner produced by mixing a toner for use in electrophotography with a charge controlling agent while applying mechanical strain force to embed the charge controlling agent in the surface of the toner (Japanese patent application No. 51481/1986). However, it was found that, even with this improved method, the desired charge control cannot be often attained depending on the formulation of the toner and the conditions of production. Specifically, when the surface of the core particles (A) is preliminary coated with an electrically conductive material such as carbon black or a surfactant, difficulties are encountered in controlling the charges even when the charge controlling agent (B) is embedded in the surface of the core particles (A) by the above-mentioned method. The reason for this has not yet been fully elucidated. In any way, as is apparent from the foregoing description, the conventional toners still present problems to be solved.

40 SUMMARY OF THE INVENTION

An object of the present invention is to solve the above-mentioned problems and to provide a toner which can be prepared with excellent productivity and can produce a clear image free from fogging.

The present inventors have made extensive and intensive studies. As a result, the present inventors have found that a toner for use in electrophotography, which is superior in productivity and sharpness in charge distribution to the conventional toners, can be stably obtained by mixing thermoplastic resin core particles (A) with carrier particles (C) having an average particle size of from 0.05 to 2.0  $\mu\text{m}$ , preferably 0.08 to 2.0  $\mu\text{m}$  and carrying a charge controlling agent (B) on the surface thereof while applying mechanical strain force under such conditions that the resulting toner particles have an average particle size of from 1 to 20  $\mu\text{m}$ , thereby embedding the carrier particles (C) in the surface of the core particles. The present invention is based on this finding. Specifically, in accordance with the present invention, there is provided a toner for use in electrophotography comprising thermoplastic resin core particles (A) or (A') and carrier powders (C) which carry a charge controlling agent (B) on the surface thereof and are embedded in the surface of said core particles (A) or (A'), said toner being produced by mixing the core particles (A) having an average particle size of from 1 to 15  $\mu\text{m}$  or the core particles (A') having an average

particle size of from 1 to 15  $\mu\text{m}$  and containing colorant particles embedded in the surface thereof, with carrier particles (C) having an average particle size of from 0.1 to 2.0  $\mu\text{m}$  and carrying a charge controlling agent (B) on the surface thereof while applying mechanical strain force to the resulting mixture under such conditions that the resulting toner particles have an average particle size of from 1 to 20  $\mu\text{m}$ . The state wherein "carrier particles (C) which carry a charge controlling agent (B) on the surfaces thereof are embedded in the surface of core particles (A)" as described herein refers to such a state that part of the carrier particles (C) are exposed on the surface of the core particle (A) without being completely buried in the core particles (A). In this state, part of the charge controlling agent (B) carried on the carrier particles (C) are exposed on the surfaces of the core particles (A). However, it is not necessary that all of the carrier particles (C) be exposed on the surfaces of the core particles (A).

In the present specification, the particle size was measured with a Coulter Counter Model TAII (a product of Coulter Electronics Co., Ltd.) and expressed on the volume basis.

#### DETAILED DESCRIPTION AND PREFERRED EMBODIMENTS OF THE INVENTION

The core particles used in the present invention may be those obtained by conventional methods, i.e., by mixing a thermoplastic resin with a coloring material and, if necessary, additives such as a lubricant, followed by being subjected to a series of procedures such as melting, kneading, allowing to cool, coarse grinding, grinding, and then classification. Alternatively, the core particles may be those obtained by embedding a coloring material substantially as a primary particle in the surfaces of resin particles through the mixing operation under the same mechanical strain force as that of the present invention. Although the colorant such as pigment exists as a secondary agglomeration, since the colorant thus obtained by mixing operation is embedded to the surface of the core particle substantially as a primary particle, colorant core particle having tinting power and brightness is obtained (see U.S. patent application No. 020,585).

Examples of thermoplastic resins for the core particles which may be used in the present invention include known binder resins, e.g., polystyrene resins, copolymer resins containing styrene, such as copolymer of styrene with acrylate, methacrylate, acrylonitrile or maleate, polyacrylate resins, polymethacrylate resins, polyester resins, polyamide resins, polyvinyl acetate resins, epoxy resins, phenolic resins, hydrocarbon resins, petroleum resins, and chlorinated paraffins. Further, it is preferred that the thermoplastic resins be solid at room temperature and have a heat softening temperature of 50° C. or higher. These may be used alone or in the form of any mixture. With respect to other additives, coloring materials such as pigment and dye, magnetic powder, lubricants such as wax, fluidizers such as colloidal silica, and low-molecular weight polyolefins may be used in combination according to the purposes. When they are used in the form of fine particles, they can be also embedded in the same manner as that described above with respect to the carrier particles (C). It is preferred that the core particles (A) be substantially free from particles having a particle size of 25  $\mu\text{m}$  or more. Although it is generally believed that fine particles having a size of 1  $\mu\text{m}$  or less are unfavorable, it is

not necessary in the present invention, as is mentioned later, that such fine particles be removed because the particle sizes are regulated by the mixing treatment.

Examples of the coloring material include white and black pigments or dyes, such as zinc yellow, yellow iron oxide, hansa yellow, disazo yellow, quinoline yellow, permanent yellow, red iron oxide, permanent red, lithol red, pyrazolone red, watchung red calcium salt, watchung red manganese salt, lake red C, lake red D, brilliant carmine 6B, brilliant carmine 3B, prussian blue, phthacyanine blue, metal-free phthacyanine, titanium white, and carbon black.

Examples of the carrier particles (C) include inorganic fine powders such as alumina, titanium dioxide, barium titanate, magnesium titanate, strontium titanate, zinc oxide, iron oxide, barium sulfate, silicon carbide, cerium oxide, silica, and carbon powder; fine particles of resins such as polyvinylidene fluoride, copolymers of vinylidene fluoride with vinyl fluoride, trifluoroethylene, ethylene, propylene, butene or the like, polystyrene, styrene-methyl methacrylate copolymer, xylene resin, polyamide, petroleum resins such as cumarone-indene resin, benzoguanamine resin, phenolic resin, melamine resin, epoxy resin, and unsaturated polyester resin; and fine particles of organic substances, e.g., waxes such as polyethylene wax and amide wax and metal salts of fatty acids, such as calcium stearate, aluminum stearate, and zinc stearate. It is preferred that these fine particles have a particle size of from 0.1 to 2.0  $\mu\text{m}$ . When the particle size is too large, the carrier particles cannot be uniformly embedded in the core particles (A). On the other hand, the particle size is too small, the carrier particles (C) are completely embedded in the inside of the core particles (A), which makes it impossible to attain the main object. Further, it is preferred that the carrier particles (C) be solid at room temperature and have a heat softening temperature of 50° C. or above.

In the present invention, although the methods of carrying the charge controlling agent (B) on the surface of the carrier particles (C) are not particularly limited, it is preferred that the charge controlling agent be deposited to attain a sufficient strength. A preferable method for attaining this purpose comprises subjecting both components to wet mixing, drying the resulting mixture and, if necessary, grinding the dried mixture. Specifically, 1 weight part of the charge controlling agent (B) and 1 to 10 weight parts of the carrier particles (C) are milled using a ball mill, a sand mill or an attritor in the presence of a suitable medium, such as water or an organic solvent, followed by drying and grinding. The resulting product can be advantageously used in the present invention.

The charge controlling agent (B) used in the present invention may be one known in the art, and examples include dyes and metal-containing dyes such as Fetschwarz HBN, Nigrosine Base, Brilliant Spirit, Zapon Black X, Ceres Black RG, copper-phthacyanine dye; other dyes such as C.I. Solvent Black 1, 2, 3, 5, and 7, C.I. Acid Black 123, 22, 23, 28, 42, and 43, Oil Black (C.I. 26150) and Spiron Black; quaternary ammonium salt; metal salt of naphthenic acid; and metallic soaps of fatty acids and resin acid. In the present invention, in mixing the core particles (A) with the carrier particles (C) carrying the charge controlling agent (B) on the surfaces through the application of mechanical strain force under such conditions that the resulting toner particles have an average particle size of from 1 to 20

μm, it is necessary that the mixing be conducted so as not to cause unfavorable phenomena such as fusion of the core particles (A) to form a large mass and grinding into finely divided particles due to the application of excessive strain force and at the same time, so as to embed part of the carrier particles (C) carrying the charge controlling agent (B) on the surfaces in the surfaces of the core particles (A). In the case of commercial scale production, both of the above-mentioned requirements can be met by varying the operating conditions of a dispenser such as a ball mill or a sand mill etc. and conditions such as loading and dispersing medium so as to attain the above-mentioned purpose.

However, the mixing step with a ball mill or a sand mill requires much time. In this respect, mixers preferable from the stand point of commercial scale production include one in which particles are fluidized together with an air stream at a high speed and one equipped with a blade or a hammer capable of applying percussions. Examples of such mixers include an SI mill (a product of Toyo Ink Mfg. Co., Ltd.; some description on an SI mill is given in Japanese patent application Publication No. 43051/1982), an atomizer, a Jiyu Mill (a product of Nara Machinery Co., Ltd.), a grinder manufactured by Kawasaki Heavy Industries, Ltd. (KTM-1), and a Hybridizer (a product of Nara Machinery Co., Ltd.). These devices may be used as they are or used after they are modified according to the purposes of the present invention. If possible, it is preferred that a hermetically sealed device of circulation type, e.g., a Hybridizer, be used.

Further, it is preferred that the core particles (A) be pre-mixed with the carrier particles (C) carrying the charge controlling agent (B) on the surfaces and other fine particles under stirring conditions milder than those of the above-mentioned mixing treatment, e.g., in a Henschel mixer. The pre-mixing causes the fine particles such as the particles (C) to be electrostatically deposited on the core particles (A), which contributes to the uniform embedding of the fine particles in the core particles (A).

The reason why the mixing treatment causes such an effect that the carrier particles (C) carrying the charge controlling agent (B) on the surfaces are embedded on the surfaces of the core particles (A) is believed to reside in that these particles come into collision with each other or with the wall, blade or dispersing medium such as beads to instantaneously and partly generate a considerably high temperature, which leads to occurrence of a phenomenon similar to a mechanical reaction in the field of inorganic chemistry. Therefore, it is sometimes necessary that the system be allowed to cool. When the air stream temperature in the system is raised to around the  $T_g$  (glass transition point) of the resin, the particles tend to fuse to each other.

The above-mentioned phenomenon can be confirmed through examination of electron photomicrograph prior to mixing treatment, i.e., after pre-mixing, and after mixing treatment. Specifically, before the mixing treatment, the core particles (A) having a relatively broad particle size distribution and the carrier particles (C) carrying the charge controlling agent (B) on the surfaces are in a partly agglomerated state. On the other hand, after the mixing treatment, the core particles (A) are in a smooth state as a result of the removal of the angular portion thereof, and it is observed that the carrier particles (C) are embedded in the surface of the core particles (A). The resulting particles were hardly

broken by the running test conducted within a copying device. Further, since the charge controlling agent (B) is present on the surface of the toner, the amount of the charge can be effectively regulated by the use of a small amount of the charge controlling agent (B).

Various factors for attaining the above-mentioned effects may be mentioned. According to the studies conducted by the present inventors, the most important factor is the speed of the air stream of the mixing devices and it is preferred that the speed of the air stream be several tens to several hundreds m/sec.

In the present invention, it is preferred that the toner particles have such a particle size distribution that they have an average particle size of from 1 to 20 μm and are free from particles having a size of 0.5 μm or less and 25 μm or more. The presence of a large amount of the toner particles having a size of 0.5 μm or less brings about a lowering in the flow, which leads to the occurrence of staining of copied paper. On the other hand, the presence of a large amount of the toner particles having a size of 25 μm or more leads to the formation of a roughened image, which brings about a reduction in the commercial value. However, the toner according to the present invention does not need any particular classification because the particles having a size of 0.5 μm or less is regulated with respect to the particle size.

In the present invention, when the production of a magnetic toner is intended, known thermoplastic resin core particles containing magnetic powders may be used. Alternatively, if necessary, core particles (A) having magnetic particles embedded therein obtained by the same procedures as those adopted in the present invention may be also used. The magnetic particles are not particularly limited. However, it is preferred that finely divided magnetic particles having an average particle size of 1 μm or less, preferably 0.5 μm or less, be used when the magnetic toner is produced by the latter method. Examples of the magnetic particles known in the art, include various ferrites, magnetite, hematite, and alloys or compounds of iron, zinc, cobalt, nickel, and manganese. These magnetic particles may be those which were subjected to classification according to the purposes or known surface treatment, e.g., hydrophobic treatment or silane coupling agent treatment.

The present invention will now be described with reference to the following examples. In the examples, all the parts are by weight.

#### REFERENCE EXAMPLE 1

100 parts of carbon powder (Sevacarb MT-CI; trade name of a product of Columbia Carbon Co., Ltd.; an average particle size of 0.35 μm), 20 parts of a charge controlling agent (PNR-BE; trademark of a product of Orient Chemical Industries, Ltd.), and 200 parts of water were mixed with each other in a ball mill for 24 hours. The mixture was filtered and then dried at 100° C. for 24 hours to obtain carrier particles (1) carrying a charge controlling agent on the surfaces of carbon powder.

#### REFERENCE EXAMPLE 2

Carrier particles (2) were produced in the same manner as that of Reference Example 1, except that Oil Black 1010 (trademark of a product of Chuo Synthetic Chemical Co., Ltd.) was used as the charge controlling agent.

## REFERENCE EXAMPLE 3

Carrier particles (3) were produced in the same manner as that of Reference Example 1, except that 100 parts of barium sulfate (B-30; trade name of Onahama Sakai Chemical Co., Ltd.; an average particle size of 0.3  $\mu\text{m}$ ), 20 parts of a charge controlling agent (PNR-BE; trademark of a product of Orient Chemical Industries, Ltd.), and 140 parts of water were used.

## REFERENCE EXAMPLE 4

Carrier particles (4) were produced in the same manner as that of Reference Example 3, except that precipitated barium sulfate 100 (trade name of a product of Onahama Sakai Chemical Co., Ltd.; an average particle size of 0.6  $\mu\text{m}$ ) was used as barium sulfate.

## REFERENCE EXAMPLE 5

Carrier particles (5) were produced in the same manner as that of Reference Example 3, except that precipitated barium sulfate 300 (trade name of a product of Onahama Sakai Chemical Co., Ltd.; an average particle size of 0.8  $\mu\text{m}$ ) was used as barium sulfate.

## REFERENCE EXAMPLE 6

Carrier particles (6) were produced in the same manner as that of Reference Example 3, except that 100 parts of the same barium sulfate as that used in Reference Example 3, 20 parts of a charge controlling agent (E-84; trademark of a product of Orient Chemical Industries, Ltd.), and 150 parts of water were used.

## REFERENCE EXAMPLE 7

Carrier particles (7) were produced in the same manner as that of Reference Example 5, except that the amounts of barium sulfate and the charge controlling agent were 100 parts and 10 parts, respectively.

## REFERENCE EXAMPLE 8

Carrier particles (8) were produced in the same manner as that of Reference Example 5, except that the amounts of barium sulfate and the charge controlling agent were 100 parts and 30 parts, respectively.

## REFERENCE EXAMPLE 9

Carrier particles (9) were produced in the same manner as that of Reference Example 2, except that particles having a size of about 0.5  $\mu\text{m}$  obtained by classification of benzoguanamine resin particles (EP-S; trade name of a product of Nippon Shokubai Kagaku Kogyo Co., Ltd.) were used instead of the carbon powder.

## EXAMPLE 1

96 parts of a styrene-acrylic resin (Nikalite NC-6100; trade name of a product of Nippon Carbide Industries Co., Ltd.) and 4 parts of low-molecular weight polypropylene (Viscol 550 P; trade name of a product of Sanyo Chemical Industry Ltd.) were mixed with each other in a Henschel mixer. The resulting mixture was molten, kneaded and allowed to cool in a twin-screw extruder. The kneading product was coarsely ground and then fed in a type I jet mill to obtain resin particles having a maximum particle size of 25  $\mu\text{m}$  or less and an average particle size of about 10  $\mu\text{m}$ .

100 parts of the resin particles and 4 parts of carbon black (Monarch 880; trade name of a product of Cabot Corporation; a particle diameter of 16 m  $\mu$ ) were pre-mixed with each other in a Henschel mixer at a circum-

ferential speed of 10 m/sec for 10 minutes to deposit carbon black on the surfaces of the resin particles. 100 g of the treated resin particles were fed into a Hybridizer (Model NHS-1). The Hybridizer was operated at 8,000 rpm for 2 minutes to obtain core particles in which the carbon black was embedded. During this step, the Hybridizer was cooled with water of 20° C.

100 parts of the core particles and 6 parts of the carrier powders (1) were subjected to the pre-mixing treatment and the mixing treatment in a Hybridizer in the same manner as that described above, thereby obtaining a toner having an average particle size of about 11  $\mu\text{m}$  and substantially free from particles having a size of 5  $\mu\text{m}$  or less and 25  $\mu\text{m}$  or more.

The amount of blow-off electrification of the toner thus obtained was  $-20 \mu\text{c/g}$ , and the measurement with a particle charge measuring device (a product of Hosokawa Micron Corporation) revealed that the toner was substantially free from toner particles having a reversed polarity.

100 parts of the toner was added and mixed with 0.3 parts of finely divided silica (R-972; trade name of a product of Nippon Aerosil Co., Ltd.). The resulting mixture was further mixed with 900 parts of an iron powder carrier to prepare a two-component developing agent. The developing agent was set within a copying machine manufactured by Toshiba Corp. (trade name: BF-8411). The copying on plain paper was continuously conducted by making use of a test chart.

In this copying test, the toner was excellent in charge stability, fixability, blocking resistance, and offset resistance and provided an image substantially free from scumming and fogging. Further, in a running test in which the copying operation was conducted while supplying the toner in a supply hopper of the copying machine, the toner was smoothly supplied, and the quality of the initial image was maintained until the image was duplicated on 60,000 pieces of plain paper.

## EXAMPLE 2

A flask was charged with 500 parts of purified water and 8 parts of polyvinyl alcohol and maintained at 80° C. under a nitrogen gas stream. 50 parts of butyl acrylate and 1 part of benzoyl peroxide were added while stirring to the flask for about 30 minutes. The resulting mixture was maintained at that temperature for 30 minutes while stirring. Thereafter, 400 parts of styrene, 50 parts of butyl acrylate, and 4 parts of benzoyl peroxide were added thereto in about 2 hours. The stirring was further continued at 80° C. for 4 hours, and the resulting product was dried at a low temperature, thereby obtaining pearl polymerization resin particles having an average particle size of 11.5  $\mu\text{m}$ . The same procedures as those of Example 1 were repeated to obtain a toner, except that the above-prepared pearl polymerization resin particles were used. The toner had an average particle size of about 12.5  $\mu\text{m}$  and an amount of blow-off electrification of  $-17 \mu\text{c/g}$  and exhibited excellent properties comparable to those of the toner as produced in Example 1.

## COMPARATIVE EXAMPLE 1

A toner was produced in the same manner as that of Example 1, except that 1 part of a charge controlling agent (PNR-BE) which had been subjected to classification to obtain particles having a size of 1  $\mu\text{m}$  was used instead of the carrier particles (1). The toner thus obtained had an amount of blow-off electrification of  $-9$

$\mu\text{c}/\text{g}$ . The toner was applied to the same test as that of Example 1. The above-obtained toner was inferior in resistance to scumming and fogging to the toners as produced in Examples 1 and 2.

#### COMPARATIVE EXAMPLE 2

A toner was produced using the same starting materials as those of Example 1 by a conventional method.

Specifically, 96 parts of a styrene-acrylic resin, 4 parts of low-molecular weight polypropylene, 4 parts of carbon black, and 3 parts of a charge controlling agent (used in an increased amount because of the incorporation method employed) were pre-mixed with each other in a Henschel mixer. The resulting mixture was molten, kneaded and allowed to cool in a twin-screw extruder, followed by coarse grinding. The coarse powders thus obtained were ground in a type I jet mill grinder and then subjected to classification to obtain a toner having a particle size of from 5 to 25  $\mu\text{m}$ . The toner was applied to the same test as that of Example 1. The above-obtained toner was inferior in resistance to scumming and fogging to the toners as produced in Examples 1 and 2 and further caused a bridging phenomenon within the toner hopper.

#### EXAMPLE 3

A toner was produced in the same manner as that of Example 1, except that the carrier particles (2) were used instead of the carrier particles (1).

The amount of blow-off electrification of the toner was obtained was +19  $\mu\text{c}/\text{g}$ , and the measurement with a particle charge measuring device (a product of Hosokawa Micron Co., Ltd.) revealed that the toner was substantially free from toner particles having a reversed polarity.

100 parts of the toner was added and mixed with 0.1 part of finely divided silica (R-972; trade name of a product of Nippon Aerosil Co., Ltd.). The resulting mixture was further mixed with 900 parts of an iron powder carrier to prepare a two-component developing agent. The developing agent was set within a copying machine manufactured by Sharp Corporation (trade name: SF8100). The duplication of an image on plain paper was continuously conducted by making use of a test chart.

In this copying test, the toner was excellent in charge stability, fixability, blocking resistance, and offset resistance and provided an image substantially free from scumming and fogging. Further, in a running test in which the copying operation was conducted while supplying the toner in a supply hopper of the copying machine, the toner was smoothly supplied, and the quality of the initial image was maintained until the image was duplicated on 60,000 pieces of plain paper.

#### EXAMPLE 4

The same procedures as those of Example 1 were repeated, except that 53 parts of a styrene-acrylic resin (Himer SMB73; trade name of a product of Sanyo Chemical Industry Ltd.), 42 parts of magnetic particles (MAT-305 HD; trade name of a product of Toda Kogyo Corporation; a particle size of 0.2  $\mu\text{m}$ ), and 3 parts of low-molecular weight polypropylene (Viscol 550P; a product of Sanyo Chemical Industry Ltd.) were used, thereby obtaining resin particles having a maximum particle size of 25  $\mu\text{m}$  or less and an average particle size of 10  $\mu\text{m}$ .

98 parts of the resin particles and 2 parts of carbon black (Monarch 880; trade name of a product of Cabot Corporation; a particle size of 16  $\mu\text{m}$ ) were subjected to the pre-mixing treatment and the mixing treatment with a Hybridizer in the same manner as that of Example 1 to obtain core particles having carbon black embedded on the surfaces thereof.

100 parts of the core particles and 6 parts of the carrier particles (3) were subjected to the pre-mixing treatment and the mixing treatment with a Hybridizer in the same manner as that of Example 1 to obtain a toner having an average particle size of about 12  $\mu\text{m}$  and substantially free from particles having a size of 5  $\mu\text{m}$  or less and 25  $\mu\text{m}$  or more.

15 The toner had an amount of blow-off electrification of -26  $\mu\text{c}/\text{g}$  and exhibited excellent charge distribution. 100 parts of the toner was added and mixed with 0.3 parts of finely divided silica (R-972; trade name of a product of Nippon Aerosil Co., Ltd.). The resulting mixture was set within a copying machine manufactured by Canon Inc. (trade name: NP300 Z). The duplication of an image on plain paper was continuously conducted by making use of a test chart.

In this copying test, the toner was excellent in charge 25 stability, fixability, blocking resistance, and offset resistance and provided an image substantially free from scumming and fogging. Further, in a running test, the toner was smoothly supplied, and the quality of the initial image was maintained until the image was duplicated on 50,000 pieces of plain paper.

#### EXAMPLE 5

Two kinds of toners were produced in the same manner as that of Example 4, except that the carrier particles (4) and the carrier particles (5) were used instead of the carrier particles (3).

These toners were applied to the same test as that of Example 4. They exhibited excellent results comparable to those of Example 4.

#### EXAMPLE 6

100 parts of the resin as used in Example 1 and 4 parts of a red azo pigment were subjected to the pre-mixing treatment and the mixing treatment in a Hybridizer in the same manner as that of Example 1, thereby obtaining core particles having a red azo pigment embedded on the surfaces thereof.

100 parts of the core particles and 6 parts of the carrier particles (6) were subjected to the pre-mixing treatment and the mixing treatment in a Hybridizer in the same manner as that of Example 1 to obtain a toner.

The toner had an amount of blow-off electrification of -24  $\mu\text{c}/\text{g}$  and exhibited excellent charge distribution.

55 100 parts of the toner was added and mixed with 0.3 parts of finely divided silica (R-972; trade name of a product of Nippon Aerosil Co., Ltd.). The resulting mixture was further mixed with 900 parts of an iron powder carrier and then set within a copying machine manufactured by Mita Industrial Co., Ltd. (trade name: DC-232). The duplication of an image on plain paper was continuously conducted by making use of a test chart. The toner exhibited excellent results comparable to those of Example 1.

#### EXAMPLE 7

A toner was produced in the same manner as that of Example 6, except that 12 parts of the carrier particles

(7) were used instead of the carrier particles (6). This toner was applied to the same test as that of Example 6. The toner exhibited excellent results comparable to those of Example 6.

## EXAMPLE 8

A toner was produced in the same manner as that of Example 6, except that 4 parts of the carrier particles (8) was used instead of the carrier particles (6). This toner was applied to the same test as that of Example 6. The toner exhibited excellent results comparable to those of Example 6.

## EXAMPLE 9

A toner was produced in the same manner as that of Example 3, except that 4 parts of the carrier particles (9) was used instead of the carrier particles (2). This toner was applied to the same test as that of Example 3. The toner exhibited excellent results comparable to those of Example 3.

What is claimed is:

1. A toner for use in electrophotography comprising thermoplastic resin core particles (A) having an average particle size of from 1 to 15  $\mu\text{m}$ , a charge controlling agent (B) and carrier particles (C) having an average particle size of from 0.05 to 2.0  $\mu\text{m}$ , the charge controlling agent (B) being carried on the surfaces of the carrier particles (C), and the carrier particles (C) with the agent (B) carried thereon being embedded in the surfaces of the resin core particles (A) by mixing the core particles (A) and the carrier particles (C) with the agent (B) carried thereon while applying mechanical strain force to the mixed materials under such conditions that the resulting toner particles have an average particle size of from 1 to 20  $\mu\text{m}$ .

2. A toner for use in electrophotography according to claim 1, wherein the carrier particles (C) with the charge controlling agent (B) carried thereon are those produced by wet mixing the charge controlling agent (B) with the carrier particles (C) having an average

5 particle size of from 0.05 to 2.0  $\mu\text{m}$  to tightly adhere the charge controlling agent (B) to the carrier particles (C).  
 3. A toner for use in electrophotography according to claim 1, wherein the thermoplastic resin core particles (A) are pre-mixed with the carrier particles (C) with the charge controlling agent (B) carried thereon under stirring conditions milder than those obtained in the mixing treatment using said mechanical strain force.  
 4. A toner for use in electrophotography according to claim 1, wherein magnetic particles are preliminarily mixed in said thermoplastic resin core particles (A).  
 5. A toner for use in electrophotography according to claim 1, wherein the colorant is preliminarily mixed in said thermoplastic resin core particles (A).  
 6. A toner for use in electrophotography comprising colorant-embedded thermoplastic resin core particles (A') having an average particle size of from 1 to 15  $\mu\text{m}$ , a charge-controlling agent (B) and carrier particles (C) having an average particle size of from 0.1 to 2.0  $\mu\text{m}$  and carrying a charge-controlling agent (B) on the surfaces thereof, the colorant being embedded in the original thermoplastic core particles by mixing the colorant and the original core particles while applying mechanical strain force to the mixed materials under such conditions that the resulting colorant-embedded core particles have an average particle size of from 1 to 15  $\mu\text{m}$ , and the carrier particles (C) with the charge-controlling agent (B) carried thereon being embedded in the colorant-embedded resin core particles (A') by mixing the resin core particles (A') and the carrier particles (C) with the agent (B) carried thereon while applying mechanical strain force to the mixed materials under such conditions that the resulting toner particles have an average particle size of from 1 to 20  $\mu\text{m}$ .

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

particle size of from 0.05 to 2.0  $\mu\text{m}$  to tightly adhere the charge controlling agent (B) to the carrier particles (C).

3. A toner for use in electrophotography according to claim 1, wherein the thermoplastic resin core particles (A) are pre-mixed with the carrier particles (C) with the charge controlling agent (B) carried thereon under stirring conditions milder than those obtained in the mixing treatment using said mechanical strain force.

4. A toner for use in electrophotography according to claim 1, wherein magnetic particles are preliminarily mixed in said thermoplastic resin core particles (A).